

Mar. 13, 1923.

1,448,036.

R. E. PEARSON ET AL.

REDUCTION OF OXIDES OF METALS OF THE CHROMIUM GROUP.

FILED JULY 12, 1921.



Inventors  
(Richard Edgar Pearson,  
Custace Neville Craig,  
John Reginald Stubbis, Benjamin Farnelle,  
their atto).

## UNITED STATES PATENT OFFICE.

RICHARD EDGAR PEARSON AND EUSTACE NEVILLE CRAIG, OF LONDON, ENGLAND,  
ASSIGNORS TO DURELCO LIMITED, OF LONDON, ENGLAND, A BRITISH COMPANY.

## REDUCTION OF OXIDES OF METALS OF THE CHROMIUM GROUP.

Application filed July 12, 1921. Serial No. 484,168.

To all whom it may concern:

Be it known that we, RICHARD EDGAR PEARSON and EUSTACE NEVILLE CRAIG, subjects of the King of England, both residing at Hanwell, London, England, have invented certain new and useful Improvements in the Reduction of Oxides of Metals of the Chromium Group, of which the following is a specification.

- 10 This invention is for improvements in or relating to the reduction of oxides of metals of the chromium-group, more particularly for use in the preparation of pressed and sintered bars and the like of these metals.
- 15 In classifying the metallic elements the term "chromium-group" is commonly used to embrace the metals, chromium, tungsten, molybdenum and uranium which have certain properties in common and where this 20 term occurs in the present specification and claims it is to be interpreted in its ordinary sense (i. e. as signifying the aforesaid metals).

Many methods have been suggested for 25 reducing the oxides of "chromium-group" metals to metallic form including reduction by powdered aluminium, by powdered zinc or by carbon, and in the case of the tungsten and the molybdenum which are used for the 30 manufacture of filaments and hooks for incandescent electric lamps, or for the contacts and other small parts of magnetos, ionic valves, and the like, the commonest method of reduction has involved the repeated or 35 long-continued passage of pure dry hydrogen over the heated oxide. Isolated suggestions have been made for the reduction of tungsten and molybdenum by electrolysis of their solutions or of their fused com- 40 pounds.

Considering the case of the methods commonly in use for the production of tungsten and molybdenum for the filaments and wires of incandescent lamps, the hydrogen reduction process referred to above is open to several objections. The heating operations and the supply of hydrogen are expensive. The metallic powder produced by the reduction may very easily be brought into a 45 condition in which it cannot be pressed into bars or sintered. Further for the said process it is essential to use the pure oxide (such

as  $WO_3$ ) free from soda, iron and the like, and it is a difficult and sometimes expensive matter to purify the metallic oxide 55 from such materials which may be injurious or disadvantageous in the subsequent treatment or use of the tungsten or molybdenum. One object of this invention is to facilitate the removal of impurities, and the production 60 of the metal in form well suited for the preparation of pressed and sintered bars or the like.

This invention comprises a process for the reduction to lower oxide of the tri-oxide of 65 a "chromium-group" metal which process consists in immersing a cathode in an intimate mixture (such as a paste) of the powdered oxide and an electrolyte in which it is insoluble (such as an aqueous solution of 70 sulphuric acid) and effecting reduction to lower oxide by passing a direct current through the mixture.

It is to be understood that the term "tri-oxide" includes both the anhydrous and the 75 hydrated forms of this oxide.

Preferably the paste of powdered oxide and electrolyte is contained in a porous pot or other cathode chamber surrounding the cathode.

The invention also comprises a process for the production of metallic powder for use in the manufacture therefrom of pressed and sintered bars and the like, consisting 85 in reducing the tri-oxide of a "chromium-group" metal as hereinabove described, washing the reduced product until substantially free from impurities, and heating the product in hydrogen in the known manner to complete the reduction.

The intimate mixture or paste may be agitated during reduction and in the case of molybdenum this is particularly advantageous.

Conveniently the cathode comprises a 95 number of acid-resisting metallic rods (say of nickel-chromium alloy). Any suitable metal may be used as cathode, but if the metal selected be soluble in the electrolyte as zinc is in sulphuric acid, the cathode and electrolyte must not be allowed to remain in contact without current passing.

The invention also comprises a method of carrying out the foregoing process in which

the anode is surrounded with a material which it is desired to oxidize and which oxidizes in preference to the anode. For example, with a lead anode, waste molybdenum may be packed around the anode, whereby the oxygen produced by the electrolysis converts the molybdenum into powdered oxide of molybdenum, which can be used for the production of fresh molybdenum powder. Lead and carbon are suitable materials for use as an anode.

The following is a description, by way of example, of one preferred method of carrying out this invention as applied to the treatment of trioxide of tungsten, the figure of the drawings being illustrative of a suitable form of apparatus.

The apparatus comprises any desired number of electrolytic cells, e. g. large rectangular jars 1 of glass or earthenware. The electrolyte is a solution of sulphuric acid of specific gravity 1.2. In each jar is a porous pot 2 for the anode and a porous pot 3 for the cathode. The anode consists of a stout rod 4 of lead. The cathode consists of a number (say about 30) of thin rods 5 of nickel-chromium alloy connected at their upper ends to a metal contact plate 6 and extending down into the cathode pot. The agitator consists of a horizontal metal ring 7 embracing the outside of the cathode rods, and connected by radial spokes 8 to a central vertical rod which can slide through the top plate 6 of the cathode. This agitator preferably forms part of the cathode.

The powdered oxide of tungsten,  $WO_3$  is mixed into a paste (like paint) with the dilute sulphuric acid and introduced into the cathode porous pot. (For example, 900 grm. of  $WO_3$  may be used with 150 cc. of dilute sulphuric acid, sp. gr. 1.2 for each pot.)

The electrodes are connected to any suitable source of direct current at a voltage of say 6 volts, which may rise slightly say to 7 volts during the process, and reduction is continued to the desired extent, the paste being stirred from time to time. The average working temperature of the reaction is between 40° C. and 60° C., depending upon the current used, a suitable current being in the nature of 30 amperes, giving a current density of 0.10 amperes per square centimetre at the cathode and 0.28 amperes per square centimetre at the anode.

It is found economical not to continue the reduction till the lowest stage of oxidation is reached but only as far as the production of a lower oxide such as  $WO_2$ , which will not readily re-oxidize when removed from the apparatus. The reduced material is washed to recover the acid and to remove impurities and then dried on a vacuum filter.

It is found that after this reducing proc-

ess the removal of impurities such as soda, iron, etc. is a simple matter. It will be understood that insoluble substances such as quartz would not be removed. The reduced powder is in a state of very fine subdivision and can readily be further reduced by heating in a current of hydrogen to a metallic powder which is peculiarly well adapted to be pressed into rods or bars and sintered.

It is found that the presence in the paste or the electrolyte of certain soluble metallic salts of which the metal is more easily oxidizable than the tungsten may be advantageous in hastening or facilitating the reaction. For example, zinc sulphate has been successfully employed.

In the anode compartment the lead anode would normally be oxidized by the oxygen evolved by the electrolysis. The anode pot may therefore be filled with a material which it is desired to oxidize and which oxidizes in preference to the lead anode. For example, scrap or waste molybdenum, such as scrap wire and the like, may be packed around the anode, and in the course of the electrolysis this molybdenum is converted into powdered oxide of molybdenum which can be used for the production of fresh molybdenum powder.

In any case, however, any oxidized lead compounds produced in the anode compartment may be readily reconverted into metallic lead.

This process dispenses with the difficult and elaborate steps at present necessary for removing soda, iron etc. from  $WO_3$ . It also effects a substantial saving in hydrogen and fuel, which are normally used in the present reduction processes. An important result of the process according to this invention is the finely divided state of the product.

It will be understood that the nature of the electrodes and of the electrolyte may be varied; various means may be employed for keeping the mixture of metallic oxide and electrolyte concentrated round the cathode; and the reduction may be carried to such an extent as may be economically suitable for the particular purpose.

What we claim as our invention and desire to secure by Letters Patent is:—

1. A process for the reduction to lower oxide of the tri-oxide of a "chromium-group" metal which consists in immersing a cathode in an intimate pasty mixture of the powdered oxide and an electrolyte in which it is insoluble, and passing a direct current through the mixture.

2. A process for the reduction to lower oxide of the tri-oxide of tungsten, which consists in immersing a cathode in an intimate pasty mixture of the powdered oxide and an electrolyte in which it is insoluble, and passing a direct current through the mixture.

3. A process for the reduction to lower oxide of the tri-oxide of a "chromium-group" metal which consists in immersing a cathode in an intimate pasty mixture of the powdered oxide and an aqueous solution of sulphuric acid and passing a direct current through the mixture. 70
4. A process for the reduction to lower oxide of the tri-oxide of a "chromium-group" metal which consists in immersing a cathode comprising a number of acid-resisting metallic rods in an intimate pasty mixture of the powdered oxide and an acid electrolyte in which the oxide is insoluble, and passing a direct current through the mixture. 75
5. A process for the reduction to lower oxide of the tri-oxide of a "chromium-group" metal which consists in immersing a cathode comprising a number of rods of nickel-chromium alloy in an intimate pasty mixture of the powdered oxide and an aqueous solution of sulphuric acid, and passing a direct current through the mixture. 80
6. A process for the reduction to lower oxide, of the tri-oxide of a "chromium-group" metal which consists in obtaining within a porous cathode chamber an intimate pasty mixture of the powdered oxide and an electrolyte in which it is insoluble, immersing a cathode in said mixture, and passing a direct current therethrough. 85
7. A process for the reduction to lower oxide, of the tri-oxide of a "chromium-group" metal which consists in immersing a cathode in an intimate pasty mixture of the powdered oxide and an electrolyte in which it is insoluble, adding to said mixture a soluble metallic salt, the metal of which is more easily oxidizable than that of the oxide to be reduced, and passing a direct current through the mixture. 90
8. A process for the reduction to lower oxide, of the tri-oxide of a "chromium-group" metal at the cathode of an electrolytic cell and the simultaneous oxidation of material at the anode, which process consists in immersing the cathode in an intimate mixture of the powdered oxide to be reduced and an electrolyte in which said oxide is insoluble, surrounding the anode with material which it is desired to oxidize and which oxidizes in preference to the anode, and passing a direct current through the cell. 95
9. A process for the reduction to lower oxide, of the tri-oxide of a "chromium-group" metal at the cathode of an electrolytic cell and the simultaneous oxidation of material at the anode, which process consists in introducing into a porous pot surrounding the cathode an intimate pasty mixture of the powdered oxide to be reduced and an electrolyte in which it is insoluble, introducing into a porous pot surrounding the anode material which it is desired to oxidize and which oxidizes in preference to the anode, and passing a direct current through the cell. 100
10. A process for the reduction to lower oxide of the tri-oxide of a "chromium-group" metal at the cathode of an electrolytic cell, and the simultaneous oxidation of molybdenum at the anode, which process consists in immersing the cathode in an intimate mixture of the powdered oxide and an electrolyte in which it is insoluble, surrounding a lead anode with waste molybdenum, and passing a direct current through the cell. 105
11. For the production from the tri-oxide of a "chromium-group" metal, of metallic powder for use in the manufacture therefrom of pressed and sintered bars, a process consisting in immersing a cathode in an intimate pasty mixture of the powdered tri-oxide and an electrolyte in which it is insoluble, passing a direct current through the mixture, washing the reduced product until substantially free from impurities and heating the product in hydrogen in the known manner to complete the reduction. 110
12. A process for the production of tungsten powder for use in the manufacture therefrom of pressed and sintered bars, which process consists in immersing a cathode in an intimate pasty mixture of the powdered tri-oxide of tungsten and an electrolyte in which it is insoluble, passing a direct current through the mixture, washing the reduced product until substantially free from impurities, and heating the product in hydrogen in the known manner to complete the reduction. 115
13. A process for the reduction to lower oxide of the tri-oxide of tungsten, which consists in immersing a cathode comprising a number of acid-resisting metallic rods in an intimate pasty mixture of the powdered oxide and an acid electrolyte in which the oxide is insoluble and passing a direct current through the mixture. 120
14. A process for the reduction to lower oxide of the tri-oxide of tungsten, which consists in immersing a cathode comprising a number of rods of nickel chromium-alloy in an intimate pasty mixture of powdered oxide and an aqueous solution of sulphuric acid, and passing a direct current through the mixture. 125
15. A process for the reduction to lower oxide of tri-oxide of tungsten, which consists in immersing a cathode in an intimate pasty mixture of the powdered oxide and an electrolyte in which it is insoluble, adding to said mixture a soluble metallic salt, the metal of which is more easily oxidizable than tungsten and passing a direct current through the mixture. 130
16. A process for the reduction to lower

oxide of the tri-oxide of tungsten at the cathode of an electrolytic cell and the simultaneous oxidation of molybdenum at the anode, which process consists in immersing the cathode in an intimate mixture of the powdered oxide and an electrolyte in which it is insoluble, surrounding a lead anode with waste molybdenum, and passing a direct current through the cell. In testimony whereof we have signed our names to this specification.

RICHARD EDGAR PEARSON.  
EUSTACE NEVILLE CRAIG.